# EUROPEAN PATENT SPECIFICATION

(11) **EP 2 242 064 B1**
(45) Date of publication and mention of the grant of the patent: **28.08.2013**
(21) Application number: 09251108.8
(22) Date of filing: 16.04.2009
(51) Int. Cl.: H01B 1/00

(54) **Electrically conductive fiber and brush**
Elektrisch leitfähige Faser und Bürste
Fibre électriquement conductrice et brosse

(43) Date of publication of application: 20.10.2010
(73) Proprietor: Teijin Limited, Osaka-shi, Osaka 541-0054 (JP)
(72) Inventor: Shirakawa, Yoshiki, Matsuyama-shi, Ehime 791-8041 (JP)
(74) Representative: Hallybone, Huw George

(56) References cited:
- EP-A- 1 655 739
- WO-A-02/45098
- DE-A1- 10 336 473

## Description

As fibers having static elimination performance, for example, conductive carbon black has hitherto been caused to be contained to impart conductive performance (patent document 1 and patent document 2). Like this, the carbon black has been widely used because of its low price and excellent conductivity. However, there has been the problem of large resistance fluctuations in the conductive resistance range of 10⁸ to 10¹² Ω /cm, namely in a so-called middle to high resistance region. This is caused by a conductivity expression mechanism of the carbon black. When the carbon black is low in concentration, it has no conductivity. However, when it exceeds a certain degree of concentration, conductivity is rapidly expressed. Accordingly, the above-mentioned conductive resistance range of 10⁸ to 10¹² Ω/cm just corresponds to between the expression of conductivity and the saturation thereof, and there has been the problem of the easy occurrence of fluctuations in conductivity of the carbon black even when the carbon black has the same concentration.

Patent document 3 discloses a "composition of fluoropolymer and dispersed conductive particulate [that] provides an electrically conductive polymeric material resistant to static charge buildup".

Patent document 4 discloses a "[m]olding composition [that] has electroconductive cellulose fibers in a polymer matrix".

Patent document 5 discloses a "conductive thermoplastic composition [that] includes a polycarbonate, a polyester, a conductive filler, an impact modifier, a transesterification quench, and glass fibers".
[Patent Document 1] JP-A-2005-194650
[Patent Document 2] JP-A-2006-9177
[Patent Document 3] EP-A-1 655 739
[Patent Document 4]DE 103 36 473 A1
[Patent Document 5]WO 02/45098

### [Disclosure of the Invention]

### [Problems That the Invention Is to Solve]

An object of the present invention is to provide a conductive polyester fiber containing conductive carbon black as a conductive substance, which fiber has small fluctuations in conductive performance and stable conductive performance.

### [Means for Solving the Problems]

The present invention relates to a conductive polyester fiber containing carbon black as a main conductive component in the polyester, wherein the carbon black is composed of a mixture of at least two kinds of the following carbon blacks (A) and (B) at an A/B ratio (by weight) of 90/10 to 10/90:
(A) A conductive carbon black having an average particle size of 20 to 70 nm and an oil absorption defined in JIS K 5101 of 100 to 600 ml/100g; and
(B) A conductive carbon black having an average particle size ratio thereof to the above-mentioned conductive carbon black (A) of from 1.1 to 3, and an oil absorption ratio thereof to the above-mentioned conductive carbon black (A) of from 0.9 to 0.2.
Here, the cross-sectional resistance value of the above-mentioned conductive fiber is preferably from 10⁸ to 10¹² Ω /cm.
Further, the conductive polyester fiber of the present invention is a sheath-core type composite fiber
and the core component contains the mixture of at least two kinds of carbon blacks (A) and (B) in an amount of 10 to 35% by weight.
Further, the sheath component may contain the mixture of at least two kinds of carbon blacks (A) and (B) in an amount of 10 to 35% by weight.
On the other hand, the conductive polyester fiber described herein may be a fiber in which the mixture of at least two kinds of carbon blacks (A) and (B) is homogeneously blended with the fiber forming polymer acting as a matrix component in an amount of 10 to 35% by weight to form the whole cross section of the fiber as a conductive component.
Next, the present invention relates to a brush using the above-mentioned conductive polyester fiber.

### [Advantages of the Invention]

The conductive polyester fiber of the present invention contains the carbon black having at least two kinds of characteristics at the time of imparting conductivity, thereby being able to provide the conductive fiber having a more stable resistance value.

### [Brief Description of the Drawings]

[Fig. 1] Fig. 1 is a schematic cross sectional view of a conductive polyester fiber of the present invention.
[Fig. 2] Fig. 2 is a schematic cross sectional view of another conductive polyester fiber of the present invention.
[Fig. 3] Fig. 3 is a schematic cross sectional view of still another conductive polyester fiber of the present invention.
[Fig. 4] Fig. 4 is a schematic cross sectional view of a further conductive polyester fiber of the present invention.

### [Description of Reference Numerals and signs]

1: Sheath Component
2: Core Component

### [Best Mode for Carrying Out the Invention]

In the conductive polyester fiber of the present invention, matrix polymers with which conductive carbon black is mixed include a polyester such as polyethylene terephthalate. These matrix polymers maybe copolymerized with a third component, and may contain a delustering agent such as titanium dioxide. For example, copolymerization of isophthalic acid or adipic acid in an amount of about 10 to 20 mol% based on the whole acid components is preferred in terms of fiber-making properties. Further, ethylene glycol may be changed to a glycol component such as trimethylene glycol, tetramethylene glycol, 1,5-pentanediol or 1, 6-hexanediol, or such a glycol component may be copolymerized.

Further, the conductive polyester fiber of the present invention is a sheath-core type composite fiber. In this case, the conductive component may be arranged in either a core or a sheath. The ratio of the conductive component is usually in the range of 10 to 20% by weight of the whole fiber in terms of fiber-making properties and cost.
When the core is formed of the conductive component, fiber-making properties and fiber strength are particularly excellent. Further, when the delustering agent is caused to be contained in the sheath polymer, excellent aesthetic properties are preferably obtained. On the other hand, when the conductive component is arranged in the sheath, it is preferred in that the value of surface resistance of the conductive fiber is equalized. A polymer other than the conductive component is herein composed of a polyester, especially polyethylene terephthalate, has good texture, excellent handling properties in a processing process and good chemical resistance. Further, although the polyester is characterized in that the stiffness of the fiber is high compared to nylon and the like, the good results of improving toner scraping properties are obtained particularly by adjusting the Young's modulus to 70 cN/dtex or more when the fiber is used as a brush used in a copying machine.

The conductive fiber of the present invention is caused to contain carbon black in order to impart conductivity. As the conductive carbon black, there can be used known one, for example, acetylene black, oil furnace black thermal black channel black, Ketchen black or carbon nanotubes. These can be usually dispersed in matrix polymers to use. As the matrix polymers, the above-mentioned various polyesters are used.

In order to obtain the conductive polyester fiber of the present invention, it is important that the carbon black used as the conductive component is a mixture of at least two or more kinds of carbon blacks each having different characteristics.
First, the average particle size of one carbon black (A) is from 20 to 70 nm, and preferably from 30 to 60 nm. When the average particle size is less than 20 nm, it is difficult to homogeneously disperse the carbon black in the matrix polymer, resulting in a decrease in process yield such as an increase in yarn breakage due to coagulation at the time of fiber making. On the other hand, when the average particle size exceeds 70 nm, a larger amount of carbon black becomes necessary for obtaining desired conductive performance, as well as the problem of yarn breakage at the time of fiber making. This is also unfavorable in cost.

Further, the oil absorption of carbon black (A), which is defined in JIS K 5101, is from 100 to 600 ml/100 g, and preferably from 150 to 300 ml/100 g. When the oil absorption is less than 100 ml/100 g, the structure of the carbon black excessively develops, resulting in a decrease in process yield such as an increase in yarn breakage due to a decrease in fluidity. On the other hand, when it exceeds 600 ml/100 g, the degree of development of the structure is low, so that a large amount of carbon black becomes necessary for expressing conductivity. This unfavorably causes a cost rise.

The above-mentioned conductive carbon black (A) can be used either alone or as a combination of two or more thereof.
Commercial products of conductive carbon black (A) include "Ketchen Black" manufactured by Mitsubishi Chemical Corporation such as "EC300J" (average particle size:39.5 nm) and "EC600JD" (average particle size:34.0 nm), "TOKABLACK(TM)" manufactured by Tokai Carbon Co., LTD. such as "#5500" (average particle size:25 nm), "#4500" (average particle size:40 nm), "#4400" (average particle size:38 nm) and "#4300" (average particle size:55 nm) and "Denka Black" manufactured by Denki Kagaku Kogyo Kabushiki Kaisha such as "FX-35" (average particle size:26 nm) and "HS-100" (average particle size:48 nm), and the like.

When the carbon black is formed of a single characteristic component, there has been the problem of the easy occurrence of fluctuations in a resistance value in a middle to high resistance region such as the conductive resistance range of 10⁸ to 10¹² Ω/cm. This is caused by a conductivity expression mechanism of the carbon black. When the carbon black is low in concentration, it has no conductivity. However, when it exceeds a certain degree of concentration, conductivity is rapidly expressed, and a further increase in the amount added results in saturation. This region just corresponds to an intermediate portion of this behavior, which causes the occurrence of fluctuations in a resistance value. In order to solve this problem, at least two or more kinds of carbon blacks each having different characteristics are blended in the present invention, thereby more stabilizing the resistance value.

That is to say, in the present invention, conductive carbon black (B) in which the average particle size ratio thereof to the above-mentioned conductive carbon black (A) is from 1.1 to 3, and the oil absorption ratio thereof to the above-mentioned conductive carbon black (A) is from 0.9 to 0.2 is blended, thereby stabilizing the conductive resistance. When the average particle size ratio is less than 1.1, there is no effect of stabilizing the conductive resistance. Accordingly, it is necessary to blend the carbon black having an average particle size ratio of 1.1 or more. On the other hand, when the ratio exceeds 3, fiber-making performance extremely decreases.
Further, for the oil absorption, when the ratio exceeds 0.9, there is little difference in the degree of development of the structure, resulting in no effect of stabilizing the conductive resistance. On the other hand, less than 0.2 does not contribute to conductivity so much, and no effect is observed.

The above-mentioned conductive carbon black (B) can be used either alone or as a combination of two or more thereof.
Commercial products of conductive carbon black (B) include "Ketchen Black" manufactured by Mitsubishi Chemical Corporation such as "EC300J" (average particle size: 39.5 nm) and "EC600JD" (average particle size: 34.0nm), "TOKABLACK(TM)" manufactured by Tokai Carbon Co., Ltd. such as "#5500" (average particle size: 25 nm), "#4500" (average particle size: 40 nm), "#4400" (average particle size: 38 nm) and "#4300" (average particle size: 55 nm) and "Denka Black" manufactured by Denki Kagaku Kogyo Kabushiki Kaisha such as "FX-35" (average particle size:26 nm) and "HS-100" (average particle size:48 nm), and the like.

Then, for the mixing ratio of conductive carbon black (A) and conductive carbon black (B), the (A)/(B) ratio (by weight) is usually from 90/10 to 10/90, and preferably from 30/70 to 70/30 although it depends on a desired resistance region. When they are blended in this range, the conductive resistance is stabilized. The reason for this is not clear at the present time. However, it is believed that the behavior of changes in electric conductivity to the amount of carbon blacks added becomes slow, compared to the case where the carbon black is singly used, by blending the carbon blacks different in particle size and structure development.

Further, the carbon black comprising the above-mentioned components (A) and (B) to be blended with the conductive component is added preferably in an amount of 10 to 35% by weight, and more preferably in an amount of 10 to 25% by weight. Less than 10% by weight results in no increase in electric conductivity, whereas exceeding 35% by weight results in poor fluidity, which is unfavorable in terms of a fiber-making process. The amount of the conductive carbon black added is appropriately adjustable depending on the kind of carbon black used.

Examples of cross sectional views of the conductive polyester fibers of the present invention are shown in Figs. 1 to 4.
Of these, Fig. 1 shows the conductive polyester fiber in which the conductive carbon black mixture comprising at least two kinds of components (A) and (B) is homogeneously blended with the polyester acting as a matrix component to form the whole cross section of the fiber as a conductive component.
Further, Figs. 2 to 4 show examples of the sheath-core type conductive composite fibers, wherein the reference numeral 1 denotes a sheath component, and the reference numeral 2 denotes a core component. Figs. 2 and 4 show examples in which a conductive component is disposed as the core component, and Fig. 3 shows an example in which a conductive component is disposed as the sheath component. When the conductive component is disposed as the core component, the core component may be in modified cross section as shown in Fig. 4. In that case, for a tapered tip portion thereof, it is necessary that the ratio of a portion in which the core component is not covered with the sheath component is 5% or less of the whole periphery of the sheath component. If the ratio of the portion in which the core component is not covered with the sheath component exceeds 5%, the core and the sheath are separated from each other, or the conductive carbon black component drops off, resulting in a high possibility of causing contamination.

In the case of the conductive polyester fiber shown in Fig. 1, the mixture of at least two kinds of the above-mentioned carbon blacks (A) and (B) is homogeneously blended with the polyester acting as a matrix component in an amount of 10 to 35% by weight to form the whole cross section of the fiber as a conductive component.
Further, in the case of the sheath-core type composite fibers shown in Figs. 2 and 4, the mixture of at least two kinds of the above-mentioned carbon blacks (A) and (B) is caused to be contained in the core component in an amount of 10 to 35% by weight.
Furthermore, in the case of the sheath-core type composite fiber shown in Fig. 3, the mixture of at least two kinds of the above-mentioned carbon blacks (A) and (B) may be caused to be contained in the sheath component in an amount of 10 to 35% by weight.

The conductive polyester fiber of the present invention has static elimination performance excellent in fiber physical properties and durability in actual use, and can be suitably used as charging brushes, static eliminating brushes and cleaning brushes incorporated in OA equipment such as copying machines and printers.
Such a brush having static elimination performance is obtained, for example, by weaving the conductive fiber of the present invention as a pile fabric, backing it with a backing agent having conductivity, and then, wrapping a pile tape cut to a width of 10 to 30 mm around a cylindrical metal rod, or simply adhering the pile fabric to a plate to make it in brush form.

### [Examples]

The present invention will be illustrated in greater detail with reference to the following examples, but the invention should not be construed as being limited thereto.

### (a) Oil Absorption

The oil absorption was measured based on JIS K 5101.

### (b) Average Particle Size

The average particle size of carbon black was measured using a laser diffraction type size distribution measuring apparatus, SALD-200V ER, manufactured by Shimadzu Corporation.

### (c) Strength and Elongation of Fiber

The strength and elongation of a fiber was measured based on JIS L 1013.

(d) Internal Electric Resistance Value between Fiber End Faces
This is hereinafter referred to as the "cross-sectional resistance value". Both ends of a fiber were cut in a cross-sectional direction to a length in a fiber axis direction of 2.0 cm, and Ag Dotite (a conductive resin paint containing silver particles; manufactured by Fuj ikura Kogyo KK) was adhered to both the cross sections of the fiber. On an electrically insulating polyethylene terephthalate film, a direct current voltage of 1 KV was applied using the Ag Dotite-adhered faces under conditions of a temperature of 20°C and a relative humidity of 40%. A current flowing between both the cross sections was determined, and the electric resistance value (Ω/cm) was calculated according to Ohm's law.

### Example 1

As conductive substances, 10 parts by weight of conductive carbon black (A) ("Denka Black FX-35" manufactured by Denki Kagaku Kogyo Kabushiki Kaisha) having an average particle size of 26 nm and an oil absorption of 220 ml/100g and 9 parts by weight of conductive carbon black (B) ("Denka Black HS-100" manufactured by Denki Kagaku Kogyo Kabushiki Kaisha) having an average particle size of 48 nm and an oil absorption of 140 ml/100g were blended with 81 parts by weight of polyethylene terephthalate copolymerized with isophthalic acid in an amount of 15 mol%. Melt extrusion was performed using this composition as a core component and polyethylene terephthalate as a sheath component at a weight ratio of 10/90 to obtain a sheath-core type composite filament yarn of 50 dtex/24 filaments having a cross section as shown in Fig. 2. This operation was repeated three times to obtain 3 composite filament yarns, for each of which the cross-sectional resistance value was measured. As a result, the resistance value was in the range of 5×10⁹ to 9×10⁹ Ω/cm to show a small variation. Thus, good results were obtained.

### Comparative Example 1

As a conductive substance, 15 parts by weight of conductive carbon black (A) ("Denka Black FX-35" manufactured by Denki Kagaku Kogyo Kabushiki Kaisha) having an average particle size of 26 nm and an oil absorption of 220 ml/100g was blended with 85 parts by weight of polyethylene terephthalate used in Example 1. Melt extrusion was performed using this composition as a core component and polyethylene terephthalate as a sheath component at a weight ratio of 10/90 to obtain a sheath-core type composite filament yarn of 50 dtex/24 filaments having a cross section as shown in Fig. 2. This operation was repeated three times to obtain 3 composite filament yarns, for each of which the cross-sectional resistance value was measured. As a result, the resistance value was in the range of 5×10⁹ to 7×10¹⁰ Ω/cm to show a variation.

### [Industrial Applicability]

The conductive fiber of the present invention contains conductive carbon black as a conductive substance, and has stable conductive performance with a small variation in its conductive performance, so that it has static elimination performance excellent in fiber physical properties and durability in actual use, and can be suitably used as charging brushes, static eliminating brushes and cleaning brushes incorporated in OA equipment such as copying machines and printers.

## Claims

1. A conductive polyester fiber containing carbon black as a main conductive component in the polyester, wherein the carbon black is composed of a mixture of at least two kinds of the following carbon blacks (A) and (B) at an A/B ratio (by weight) of 90/10 to 10/90:
(A) A conductive carbon black having an average particle size of 20 to 70 nm and an oil absorption defined in JIS K 5101 of 100 to 600 ml/100g; and
(B) A conductive carbon black having an average particle size ratio thereof to said conductive carbon black (A) of from 1.1 to 3, and an oil absorption ratio thereof to said conductive carbon black (A) of from 0.9 to 0.2,
wherein the conductive polyester fiber is a sheath-core type composite fiber,
and wherein the core component of the sheath-core type composite fiber contains the mixture of at least two kinds of carbon blacks (A) and (B) in an amount of 10 to 35% by weight.

2. The conductive polyester fiber according to claim 1, wherein the cross-sectional resistance value is from 10⁸ to 10¹² Ω/cm.

3. A brush using the conductive polyester fiber according to claim 1 or claim 2.

## Patentansprüche

1. Leitfähige Polyesterfaser, die als hauptsächliche leitende Komponente in dem Polyester Ruß enthält, wobei der Ruß aus einer Mischung von mindestens zwei Arten der folgenden Ruße (A) und (B) in einem A/B-Gewichtsverhältnis von 90/10 bis 10/90 besteht:
(A) einem leitfähigen Ruß mit einer durchschnittlichen Teilchengröße von 20 bis 70 nm und einer Öladsorption gemäß JIS K 5101 von 100 bis 600 ml/100 g; und
(B) einem leitfähigen Ruß mit einem Verhältnis der durchschnittlichen Teilchengröße davon zu dem leitfähigen Ruß (A) von 1,1 bis 3,0 und einem Öladsorptionsverhältnis davon zu dem leitfähigen Ruß (A) von 0,9 bis 0,2,
wobei es sich bei der leitfähigen Polyesterfaser um eine Verbundfaser vom Kern-Mantel-Typ handelt und wobei die Kernkomponente der Verbundfaser vom Kern-Mantel-Typ die Mischung von mindestens zwei Arten von Rußen (A) und (B) in einer Menge von 10 bis 35 Gew.-% enthält.

2. Leitfähige Polyesterfaser nach Anspruch 1, wobei der Querschnittswiderstandswert 10⁸ bis 10¹² Ω/cm beträgt.

3. Bürste unter Verwendung der leitfähigen Polyesterfaser nach Anspruch 1 oder Anspruch 2.

## Revendications

1. Fibre de polyester conductrice contenant du noir de carbone comme composant conducteur principal dans le polyester, le noir de carbone étant composé d'un mélange d'au moins deux types des noirs de carbone (A) et (B) suivants dans un rapport (en poids) A/B de 90/10 à 10/90 :
(A) un noir de carbone conducteur ayant une taille moyenne de particule de 20 à 70 nm et une absorption d'huile définie en GIS K 5101 de 100 à 600 ml/100 g ; et
(B) un noir de carbone conducteur ayant un rapport entre la taille moyenne de particules de celui-ci et ledit noir de carbone conducteur (A) de 1,1 à 3, et un rapport entre l'absorption d'huile de celui-ci et ledit noir de carbone conducteur (A) de 0,9 à 0,2,
la fibre de polyester conductrice étant une fibre composite de type gaine-âme,
et le composant âme de la fibre composite de type gaine-âme contenant le mélange d'au moins deux types de noirs de carbone (A) et (B) dans une quantité de 10 à 35 % en poids.

2. Fibre de polyester conductrice selon la revendication 1, **caractérisée en ce que** la valeur de résistance transversale est de 10⁸ à 10¹² Ω/cm.

3. Brosse utilisant la fibre de polyester conductrice selon la revendication 1 ou la revendication 2.
